

Nov. 22, 1932.

F. K. WICKEL  
QUILL LIKE STRUCTURE IN THE FORM OF A RIGID, WATERPROOF,  
AND IF DESIRED, TRANSPARENT TUBE  
Filed Aug. 20, 1928

1,888,898

Fig. 1



Fig. 2



Fig. 3



Fig. 4



Fig. 5



Fig. 6



Inventor  
Frederick Karl Wickel  
By Knight Bros.  
Attorneys.

## UNITED STATES PATENT OFFICE

FRIEDRICH KARL WICKEL, OF DRESDEN, GERMANY

## QUILL-LIKE STRUCTURE IN THE FORM OF A RIGID, WATERPROOF, AND IF DESIRED, TRANSPARENT TUBE

Application filed August 20, 1928, Serial No. 300,954, and in Germany August 22, 1927.

My invention relates to a quill-like structure in the form of a rigid, waterproof, and, if desired, transparent tube, which may be used for drinking purposes, as well as for 5 a substitute for natural quills, for instance, for cigar holders, fine brushes and the like.

For drinking purposes it has already been proposed to manufacture tubes of absorbent paper saturated or impregnated with paraffin, resin emulsions and the like. Such tubes 10 cannot fulfill their object in entirely successful manner as no perfect sealing of the seams or windings is attainable. One reason is that the said impregnating materials are applicable 15 either in the melted or fused state only and possess by themselves no great adhesive-ness (such as paraffin, wax or the like) or if employed, for instance as resin emulsions they dissolve again in water and thus unroll 20 in use and become prematurely useless. The main reason is, however, that a paper to be impregnated must be naturally absorbent. The impregnating medium must thus be very thin in order that it may be absorbed at all 25 by the substance of the tube. The material of the tube absorbs the impregnating medium by capillary action and too little of the medium remains on the comparatively rough surface of the tube to suffice for an efficient 30 sealing as required for practical use. The impregnation itself calls for comparatively large quantities of material for the purpose of making the paper waterproof, so that such a process is, furthermore, expensive without 35 giving a useful result. The paraffin and its homologues are also soluble in hot water and weakly alcoholic beverages, which is, of course undesirable for taste and other reasons. Such products do not possess any 40 elasticity and are very sensitive and unable to withstand even a light lateral pressure.

According to my invention all these draw-backs are eliminated and by my improved process it is possible to produce extremely 45 elastic, very rigid, perfectly waterproof tubes capable of sustaining a high lateral pressure in a simple and less expensive manner than heretofore.

According to my invention non-absorbent 50 papers, preferably transparent papers (for

instance highly calendered sulphide cellulose papers and the like), are used in such a manner, that they receive a coating on both sides formed freely on their surfaces and remaining thereon of a material or substance preferably dissolved in a volatile solvent, which serves as a sealing, stiffening and adhesive medium. The coating substance must be odorless and tasteless. Suitable substances of this kind are, for instance, certain resins 60 dissolved in the manner of shellac in alcohol or the like, or certain artificial resins or hardening products of condensation.

As particularly suitable for the purpose has proved a condensation product of carbamide and formaldehyde. Such substances may be applied to the surfaces of the smooth and non-absorbent papers in extremely thin layers, and thus are very rational and economical. In comparison with impregnating 70 media about one tenth by weight is sufficient. The practical result of this procedure is excellent, for the reason that these materials become effective in the pure state, although in an extremely thin film. The resistance 75 against water and alcoholic or acid liquids, the natural elasticity and rigidity, on the one hand of the paper and on the other hand of the adhesive, remain unchanged. Both factors add their respective properties and 80 since, furthermore, the entire available surface of the raw material is used for adhesive purposes a product of extraordinary strength is obtained. If a naturally transparent material is employed, the tube produced possesses 85 the transparency and the character of a quill, as a substitute for which and other articles it is intended.

The layers of resin, artificial resin and the like may be applied in any desired manner. 90 The strips or webs of paper may, for instance, be provided with such coats on both sides and dried, and then during the formation and sealing of the tube exposed to heat or temporary liquefaction or the temporary softening and stickiness is obtained by a one-sided action of the solvent of the respective resin, or artificial resin covering. Another way of carrying out my improved process is to prepare only one side of the paper prior to the 100

formation of the tube, to cut the web of paper into strips, and to apply the impregnating medium to the still free side of the paper while the paper is in the machine for forming the tube, i. e. directly before the tube is constructed by coiling the paper.

In principle I claim all substances which have the property of forming waterproof, rigid and adhesive layers on papers which 10 are naturally non-absorbent or which have been made non-absorbent. By "non-absorbent" paper I mean paper which will not absorb the resinous solutions applied to it in making the tubes. Because of the extremely 15 colloidal nature of these resinous solutions which I employ, many grades of paper which will absorb melted paraffin will not absorb such resinous solutions and are therefore suitable for making tubes in accordance with my 20 invention. It is, of course, necessary to use for the coating material a substance free of taste or odor. As particularly useful for the purpose have proved condensates of carbamide and formaldehyde, the processes of 25 manufacture of which are immaterial for my invention. In their lower condensation stages they form treacle-like liquids, which may be applied in easily drying thin layers and which after the drying and heating form 30 a vitreous mass insoluble in all solvents, free of taste and smell. This and all analogous modifications by means of analogous or homologous substances form a special feature covered by a special claim.

35 The construction or formation of the tubes or tubular structures may be effected in any known or desired manner. One method of making the tube is illustrated in the drawing.

Fig. 1 is a longitudinal section through a 40 strip of raw paper, in exaggerated thickness, Fig. 2 is a longitudinal section correspond-

ing to Fig. 1, with a coating applied to the paper, likewise in exaggerated thickness,

Fig. 3 shows two paper strips cut from the 45 raw material shown in Fig. 2, in cross-section and in exaggerated thickness. The strips are shown in the relative positions in which they are wound, the upper one having its coating on top and the lower one having 50 it on the bottom,

Fig. 4 is a longitudinal section of a portion of a tube made in accordance with the invention, in greatly exaggerated thickness,

Fig. 5 is a transverse section of the tube 55 shown in Fig. 4, likewise in greatly exaggerated thickness, and

Fig. 6 shows a portion of a finished drinking tube in substantially natural thickness.

In the drawing, *a* is the raw paper, from 60 which the tubes are made and *b* is a coated layer, preferably of a condensate of carbamide and formaldehyde. From this raw material strips are cut, which are wound upon one another in the relative positions shown in 65 Fig. 3, with the coating layer of one on top

and the coating layer of the other on the bottom. A cementing layer *c* is inserted between the two layers of paper and the finished product is a tube, such as shown in Figs. 4-6. The inner and outer layers *b*, together with 70 the cementing layer *c*, seal the paper layers against penetration by liquids. The coatings *b* are relatively thin, as compared with the thickness of the paper *a*.

The new product may be produced in natural color or tinted in any shade, and decorated and inscribed as desired. It may be produced in large quantities and should be looked upon as a considerable technical improvement, as a perfect substitute for and 80 improvement on straws, quills and the like natural products.

Various changes and modifications may be made without departing from the spirit of my invention and the appended claims and I 85 desire therefore that only such restrictions should be placed upon it as are imposed by the prior art.

I claim as my invention:—

1. As a new article of manufacture, a 90 drinking tube composed of a non-absorbent paper coated with an odorless and tasteless resin.

2. As a new article of manufacture, a 95 drinking tube composed of a transparent non-absorbent paper coated with an odorless and tasteless resin.

3. As a new article of manufacture, a 100 drinking tube composed of a plurality of layers of a non-absorbent paper coated and united by an adhesive, odorless, and tasteless resin.

4. As a new article of manufacture, a 105 drinking tube composed of a non-absorbent paper coated with a hardened condensate of carbamide and formaldehyde.

5. As a new article of manufacture, a 110 drinking tube composed of a non-absorbent paper coated with a hardened condensate of carbamide and formaldehyde or its analogues or homologues.

6. As a new article of manufacture, a tubular, quill-like structure composed of a non-absorbent paper coated with a synthetic resin.

I affix my signature.

FRIEDRICH KARL WICKEL.

115

120

125

130